

Feb. 10, 1925.

1,525,518

W. H. SMITH ET AL

METHOD OF MAKING CHROMIUM CONTAINING ALLOYS

Filed Sept. 11, 1922

Fig. 1.



Fig. 2.



Fig. 3.



INVENTORS.

William H. Smith  
Charles M. Campbell

BY

Harold Elmer Smith  
ATTORNEY.

Patented Feb. 10, 1925.

1,525,518

# UNITED STATES PATENT OFFICE.

WILLIAM H. SMITH, OF CLEVELAND, AND CHARLES M. CAMPBELL, OF EAST CLEVELAND, OHIO, ASSIGNORS TO PIONEER ALLOY PRODUCTS COMPANY, OF CLEVELAND, OHIO, A CORPORATION OF DELAWARE.

## METHOD OF MAKING CHROMIUM CONTAINING ALLOYS.

Application filed September 11, 1922. Serial No. 587,300.

To all whom it may concern:

Be it known that we, WILLIAM H. SMITH and CHARLES M. CAMPBELL, citizens of the United States, residing, respectively, at 5 Cleveland and East Cleveland, in the county of Cuyahoga and State of Ohio, have invented certain new and useful Improvements in Methods of Making Chromium Containing Alloys, of which the following 10 is a specification, reference being had to the accompanying drawing.

This invention relates to a method of producing a non-corrodible alloy containing only elements of low and intricate value, 15 which alloy shall be sufficiently soft and tractable to enable it to be turned, cut, threaded and otherwise machined. It has long been known that certain alloys of chromium with iron group metals offer a 20 very high degree of resistance to corrosion, whether at ordinary atmospheric temperatures by water and ordinary gases, or at high temperatures as in furnaces and the like, or on contact with chemical reagents; 25 but difficulty has always been experienced in the preparation of these alloys due to their propensity to absorb carbon, silicon and other injurious elements which serve to increase their hardness to a point which pre- 30 cludes mechanical fabrication and increasing the brittleness to a point which frequently causes them to break upon cooling or lapse of time. Numerous prophesies have 35 been made that if an alloy of chromium and iron could be produced excluding the carbon, silicon, and other injurious ingredients, the same would be very soft, uniform, and easy to machine, and such alloys, when produced in small quantities under strict labor- 40 atory methods with pure ingredients, have confirmed the prophesy, but it has hitherto been impossible to repeat the demonstration under production conditions because of the avidity of chromium and its alloys for 45 carbon which at high temperature causes it to decompose even carbon monoxide, and to absorb carbon from the electric arc; while its avidity for silicon is such as to cause it to decompose silica either inside the 50 furnace or in the mold wherein the same is cast. Both these difficulties are enhanced by the high melting temperature of the alloy, which requires long continued heating for complete fusion, and at these high

temperatures the chromium exhibits enhanced chemical activity. Thus, a high chromium alloy if thoroughly molten and brought into contact with silica sand gives rise to a reaction accompanied by bubbling and frothing which frequently causes the mixture to spout out of the mold, and almost always leaves the castings porous and worthless.

In our former application filed August 22, 1921, Serial No. 494,055 we described and claimed a method of producing these alloys in an electric furnace of the arc type wherein the molten bath is always shielded from the arc by the interposition of an unbroken slag layer which is electrically conductive at the high temperature involved. We have discovered, however, that while it is possible to secure small and simple castings directly by this process, it is not feasible to secure larger and intricate castings in this way, since if the temperature be forced sufficiently high to produce a degree of fluidity of the molten bath necessary for the production of such a casting, the arc will almost certainly puncture the slag and so contaminate the bath as a result of dissolved carbon that the casting will be hard to machine. Furthermore the constant variation in temperature required when the same furnace is employed both for melting the alloy and bringing it to the casting point necessitates a constant variation in the composition of the slag which is difficult to effect.

According to our invention, we employ two furnaces in series, the first an arc furnace wherein is performed the process described and claimed in our application Serial No. 494,056; the second, an induction furnace which receives the molten alloy from the first furnace and elevates the temperature of same to the degree necessary for successful casting without the possibility of carbon contamination and incidentally eliminates the non-metallic impurities. In this way the first furnace can conveniently be operated within a sufficiently small range of temperature to enable the use of a slag of one composition, and with a minimum of injury to the hearth and walls; while the second furnace merely receives the molten metal at the temperature most conveniently maintained in the first furnace and boosts

this temperature quickly to the pouring temperature with a minimum current expenditure and minimum alloy contamination. Small metallic additions such as 5 tungsten, molybdenum, zirconium, manganese, and the like are also preferably added in this second furnace.

In the drawing accompanying and forming a part of this application we have shown 10 somewhat diagrammatically the steps of our improved process; Fig. 1 represents the arc furnace with its charge prior to melting; Fig. 2 illustrates the same furnace with its charge molten; and Fig. 3 represents an 15 induction furnace with its charge.

1 represents the hearth of the arc furnace, 2—2 the electrodes, which are located entirely above the surface of the metal bath. The iron is thrown or piled in the center 20 of the hearth as shown at A, the nickel (when used) around it as shown at B, and the ferrochrome around that as shown at C, the last being kept out of contact with the electrodes and covered with a mixture of lime and 25 fluorspar D, some three or four inches deep. This lime and fluorspar must be of good quality, mixed thoroughly together in the proportion of about 80% to 90% of lime and the balance fluorspar. The furnace is 30 then started in the usual manner and as soon as the iron has melted the heat thereof slowly causes the ferro-chrome to dissolve therein and the slag to soften and flow thereover so that the arc can no longer 35 strike through the slag into contact with the molten mass. This is rendered possible by the fact that the slag becomes conducting under the temperature of the electric arc. The preferred slag contains about 90% 40 lime and 10% fluorspar.

As soon as the metal has been brought to a condition of uniform composition it is drawn into the second furnace which is 45 preferably of the induction type for the reason that the latter produces its heat entirely without the use of carbon. We have found the best plan to be to employ an initial furnace of much greater capacity than the booster furnace, this maintaining 50 an amount of molten alloy continuously in the first furnace, each pour being immediately replenished by the necessary quantity of iron and ferrochrome, with or without nickel. Only a short time and small 55 expenditure of current is required to elevate

the temperature to the pouring degree in the second furnace. The alloy is cast in molds of any suitable or desired type and material excepting that we prefer to employ one which contains no silica. 60

We do not limit ourselves to the described method of charging the furnace as we can equally well build the iron on top of the ferrochrome; neither do we limit ourselves to any fixed relative sizes between the 65 furnaces, nor to a process of drawing off only a part of the alloy from the first furnace, nor in any other way except as recited in the annexed claims.

Having thus described our invention what 70 we claim is:

1. The process of producing alloys of chromium with one or more iron-group metals which contains the steps of melting the chromium and iron-group metals in a 75 preliminary arc furnace, at a comparatively low temperature beneath an electrically conducting, carbon-free slag, transferring the molten alloy to an induction furnace and there raising it to a pouring temperature 80 under neutral conditions.

2. The process of producing low-carbon alloys of chromium with iron-group metals, which contains the steps of melting the iron group metals in an electric arc furnace in 85 direct contact with the arc, adding the chromium together with a carbon-free electrically conducting slag, transferring the molten alloy to a second furnace at a temperature only slightly above fusion, and 90 heating the charge in the second furnace to a pouring temperature out of contact with carbon.

3. The process of producing low-carbon alloys containing chromium and iron-grup metals, which contains the steps of melting the essential ingredients in an arc furnace at a comparatively low temperature beneath an electrically conducting carbon-free slag, transferring the same to an induction 100 furnace, at a temperature only slightly above fusion, adding further ingredients in said induction furnace, elevating the temperature therein to that of casting, and finally casting from said second furnace. 105

In testimony whereof, we hereunto affix our signatures.

WILLIAM H. SMITH.  
CHARLES M. CAMPBELL.